

1

2,842,458

## LOW TEMPERATURE VITREOUS COATINGS FOR STEEL

Edward J. Feeney and Ernest M. Hommel, Pittsburgh, Pa., assignors to The O. Hommel Company, Pittsburgh, Pa., a corporation of Pennsylvania

No Drawing. Application May 28, 1954  
Serial No. 433,270

19 Claims. (Cl. 117—70)

This invention relates to low temperature vitreous coating of steel. More particularly the invention relates to improved vitreous coatings which may be applied at low temperatures while avoiding the scaling, the warping, the formation of gas bubbles and the necessity of coating thin sheet steel on both sides.

A large number of household appliances and building materials made of comparatively thin sheet steel are now in use which have vitreous enamel coatings. The enamel coatings are fused on the sheet steel at comparatively high temperatures, i. e. from 1400° to 1700° F. This high temperature heating of sheet steel encounters many problems which cause many coated plates to be rejected on account of imperfections. When thin sheet steel is heated at temperatures of 1300° or above the steel sags and warps and excessive oxidation occurs. This oxidation will take place on a bare sheet or under the enamel of a sheet of steel coated with a slip or enameling compound. At these high temperatures 4 to 5 mils are required in order to provide a glass that will dissolve or absorb the iron oxide being formed. Further this amount of enamel is generally applied to both sides of the steel sheet to keep it from warping.

When sheet steel is heated between 1200° and 1300° F. gaseous hydrogen is set free from the sheet surface. Also moisture in the slip and on the steel react with carbon in the steel when heated at temperatures of 1200° to 1500° F. to produce carbon gases which may generate bubbles in the enamel coating.

If sheet steel is heated in the temperature range of 850° to 1100° F. substantially no sagging, warping or oxidation occurs and comparatively few gases are released from the surface of the sheet. Most of the chemical reactions which take place when sheet steel is heated from 1400° to 1700° F. do not occur when the steel is heated to temperatures below 1200° F. At temperatures below 1200° F. it is not necessary to coat both sides of a sheet of steel to avoid warpage or the formation of gas bubbles and satisfactory coating may be obtained when using 1 to 3 mils of enamel thickness. Some articles such as steel sash and window frames as made have hollow parts which cannot be coated inside. It is important therefore to be able to coat such articles on the outside only without warpage. In fact very thin sheets of steel which cannot be satisfactorily coated with vitreous enamel at temperatures of 1400° to 1700° F. can be satisfactorily coated by the process and vitreous enamel of the present invention.

We have found that excellent hard, uniform enamel coatings which have good bonds or adherence may be obtained when the enameling operation is carried out at temperatures of 850° to 1100° F. At these low temperatures the enameled sheets may be bent without chipping and coatings may be obtained which are acid, alkali, and weather-resistant. Further the low temperature enameling operation permits a better control of the character of the surface gloss or lack of gloss than the high temperature enameling process.

2

These improved results are obtained by new enameling compounds or slips which may be made in any desired coloring and which are flexible and adhere so well to the steel that they do not chip off.

5 The primary object of the present invention is to provide a vitreous enamel suitable for producing a fused enamel coating on ferrous alloys at temperatures below 1200° F.

Another object of the invention is to provide a process 10 by which ferrous metal alloys having a coefficient of expansion in the range of 12 to  $14 \times 10^{-6}$  may be given a fused enamel coating when treated at temperatures in the range of 850° to 1100° F., which temperatures are much lower than the temperatures now being used by the trade for enameling steel.

A further object of the invention is to provide a process 15 of coating sheet steel articles with a fused vitreous enamel at temperatures below 1200° F. to provide a coated article which is alkali, acid and weather-resistant.

20 A further object of the invention is to provide a stable enameling composition which can be prepared ready for application to steel such that it may be retained in its prepared state for a long period of time and be satisfactory for use.

25 With these and other objects in view the invention consists in the new enameling composition and the process of enameling steel wares with the composition as herein-after described and particularly defined in the appended claims.

30 The present invention has a large application for the purpose of coating ferrous alloys such as steel, cast iron, wrought iron, and the many forms of stainless steel which contain more than 20% of iron. As outlined above, it is important to be able to put a continuous vitreous 35 enamel coating on various metals, particularly thin ferrous metals.

In carrying out the present invention, two types of frits are used. One frit is preferably used for coating the raw metal, and another frit of comparable composition 40 is used for the cover coat. The compositions of these two types of frits have been carefully worked out and tested to obtain glass frits which have thermal linear coefficients of expansion within  $1 \times 10^{-6}$  of the coefficients of expansion of the ferrous alloys to be coated, and particularly with sheet steels which are extensively used in the manufacture of appliances such as refrigerators, stoves, and the like.

45 Seven ground coat frits are shown in Table I.

### GROUND COAT FRITS.—PERCENTAGE BY WEIGHT

Table I

|                                | a    | b    | c    | d    | e    | f    | g    |
|--------------------------------|------|------|------|------|------|------|------|
| 55                             |      |      |      |      |      |      |      |
| Na <sub>2</sub> O              | 11.4 | 10.8 | 10.7 | 12.4 | 11.9 | 15.3 | 14.5 |
| K <sub>2</sub> O               | 2.3  | 2.2  | 2.2  | 3.5  | 3.3  | 0.5  | 2.1  |
| Li <sub>2</sub> O              | 2.2  | 2.1  | 2.0  | 1.9  | 1.9  | 0.5  | 1.0  |
| Al <sub>2</sub> O <sub>3</sub> |      |      |      |      |      | 1.0  |      |
| B <sub>2</sub> O <sub>3</sub>  | 6.9  | 10.2 | 6.5  | 7.0  | 6.7  | 13.8 | 9.5  |
| 60                             | 26.6 | 25.1 | 24.9 | 28.5 | 27.1 | 31.9 | 31.5 |
| SiO <sub>2</sub>               |      |      |      |      |      |      |      |
| F <sub>2</sub>                 | 2.0  | 2.8  | 1.8  | 4.2  | 4.0  | 1.8  | 4.7  |
| TiO <sub>2</sub>               |      |      |      |      |      |      | 2.3  |
| PbO <sub>2</sub>               | 38.4 | 36.2 | 36.0 | 34.5 | 32.9 |      | 18.3 |
| MgO                            | 6.2  | 6.8  | 3.7  | 4.4  | 4.3  |      |      |
| CaO                            | 1.1  | 1.1  | 0.7  | 0.8  | 3.4  | 13.2 | 6.8  |
| BaO                            |      |      |      | 8.8  |      | 12.3 | 6.3  |
| ZnO                            |      |      |      |      |      | 3.6  | 1.9  |
| 65                             |      |      |      |      |      |      |      |
| P <sub>2</sub> O <sub>5</sub>  |      |      |      |      |      | 1.0  |      |
| CuO                            | 1.9  | 1.8  | 2.7  | 2.8  | 2.7  |      | 3.4  |
| NiO                            | 1.0  | 0.9  |      |      |      | 1.8  |      |
| Co <sub>3</sub> O <sub>4</sub> |      |      |      |      |      | 0.9  |      |

70 This same series of ground coat frits are shown in Table II in which the parts by weight are expressed in mol percentages.

**3**  
**MOL. PERCENT**

*Table II*

|                                | <i>a</i> | <i>b</i> | <i>c</i> | <i>d</i> | <i>e</i> | <i>f</i> | <i>g</i> |
|--------------------------------|----------|----------|----------|----------|----------|----------|----------|
| Na <sub>2</sub> O              | 15.0     | 13.9     | 15.0     | 16.3     | 14.9     | 16.4     | 17.3     |
| K <sub>2</sub> O               | 2.0      | 1.9      | 2.0      | 3.0      | 2.8      | 0.4      | 1.7      |
| Li <sub>2</sub> O              | 6.0      | 5.5      | 6.0      | 5.2      | 4.8      | 16.8     | 2.6      |
| Al <sub>2</sub> O <sub>3</sub> |          |          |          |          |          | 0.6      |          |
| B <sub>2</sub> O <sub>3</sub>  | 8.0      | 11.7     | 8.0      | 8.1      | 7.5      | 13.1     | 10.0     |
| SiO <sub>2</sub>               | 35.7     | 33.4     | 36.0     | 38.1     | 35.3     | 33.1     | 38.7     |
| F <sub>2</sub>                 |          |          |          |          | 3.7      | 8.3      | 4.7      |
| TiO <sub>2</sub>               | 2.0      | 2.8      | 2.0      | 4.2      | 3.9      |          | 2.1      |
| PbO                            | 14.0     | 13.0     | 14.0     | 12.4     | 11.5     | 0.0      | 6.0      |
| MgO                            | 12.5     | 13.5     | 8.0      | 8.8      | 8.2      | 0.0      |          |
| CaO                            | 1.7      | 1.5      | 1.0      | 1.1      | 4.8      | 15.6     | 9.0      |
| BaO                            |          |          | 5.0      |          |          | 5.2      | 3.0      |
| ZnO                            |          |          |          |          |          | 3.0      | 1.7      |
| P <sub>2</sub> O <sub>5</sub>  |          |          |          |          |          | 0.5      |          |
| CuO                            | 2.0      | 1.8      | 3.0      | 2.8      | 2.6      |          | 3.2      |
| NiO                            | 1.1      | 1.0      |          |          |          | 1.6      |          |
| Co <sub>3</sub> O <sub>4</sub> |          |          |          |          |          | 0.2      |          |

By reference to Table II it will be seen that the range of variation of the constituents in the various ground coat frits is shown in Table III.

**GROUND COATS MOL PERCENTAGE***Table III*

|                                |              |
|--------------------------------|--------------|
| Na <sub>2</sub> O              | 13.9 to 17.3 |
| K <sub>2</sub> O               | 0.4 to 3.0   |
| Li <sub>2</sub> O              | 0.0 to 6.0   |
| B <sub>2</sub> O <sub>3</sub>  | 7.5 to 13.1  |
| SiO <sub>2</sub>               | 33.4 to 38.7 |
| CaO                            | 1.0 to 15.6  |
| CnO                            | 0.0 to 3.2   |
| MgO                            | 0.0 to 13.5  |
| TiO                            | 0.0 to 4.2   |
| PbO <sub>2</sub>               | 0.0 to 14.0  |
| Al <sub>2</sub> O <sub>3</sub> | 0.0 to 0.6   |
| F <sub>2</sub>                 | 0.0 to 8.3   |
| PbO                            | 0.0 to 14.0  |
| BaO                            | 0.0 to 5.2   |
| ZnO                            | 0.0 to 3.0   |
| P <sub>2</sub> O <sub>5</sub>  | 0.0 to 0.5   |
| NiO                            | 0.0 to 1.6   |
| Co <sub>3</sub> O <sub>4</sub> | 0.0 to 0.2   |

In Table IV are shown the compositions of four different frits which are suitable for use as cover coats.

**CALCULATED MELTED COMPOSITIONS FOR COVER COAT FRITS.—WEIGHT PERCENT***Table IV*

|                                | <i>A</i> | <i>B</i> | <i>C</i> | <i>D</i> |
|--------------------------------|----------|----------|----------|----------|
| Na <sub>2</sub> O              | 11.4     | 10.7     | 11.3     | 9.2      |
| K <sub>2</sub> O               | 2.3      | 2.2      | 2.3      | 1.8      |
| Li <sub>2</sub> O              | 2.1      | 2.0      | 2.1      | 1.8      |
| B <sub>2</sub> O <sub>3</sub>  | 6.9      | 6.5      | 6.8      | 9.2      |
| SiO <sub>2</sub>               | 26.6     | 24.9     | 26.3     | 23.0     |
| F <sub>2</sub>                 |          |          | 4.6      |          |
| TiO <sub>2</sub>               | 2.0      | 1.8      | 2.0      | 6.4      |
| PbO                            | 38.5     | 36.0     | 14.1     | 32.1     |
| MgO                            | 6.2      | 3.7      | 12.7     | 6.4      |
| CaO                            | 1.1      | 0.7      | 1.7      |          |
| BaO                            | 2.9      | 11.5     | 1.7      | 4.6      |
| Sb <sub>2</sub> O <sub>3</sub> |          |          | 0.3      | 0.9      |

The compositions shown in Table IV are expressed in mol percentages in Table V.

**MOL PERCENT***Table V*

|                                | <i>A</i> | <i>B</i> | <i>C</i> | <i>D</i> |
|--------------------------------|----------|----------|----------|----------|
| Na <sub>2</sub> O              | 15.2     | 15.2     | 15.1     | 11.2     |
| K <sub>2</sub> O               | 2.0      | 2.0      | 2.0      | 1.4      |
| Li <sub>2</sub> O              | 6.0      | 6.0      | 6.0      | 4.6      |
| B <sub>2</sub> O <sub>3</sub>  | 8.1      | 8.2      | 8.1      | 10.0     |
| SiO <sub>2</sub>               | 36.5     | 36.5     | 36.4     | 28.9     |
| F <sub>2</sub>                 |          |          | 12.4     |          |
| TiO <sub>2</sub>               | 2.0      | 2.0      | 2.0      | 6.1      |
| PbO                            | 14.2     | 14.2     | 14.1     | 10.9     |
| MgO                            | 12.7     | 8.1      | 12.7     | 12.0     |
| CaO                            | 1.7      | 1.2      | 1.7      |          |
| BaO                            | 1.6      | 6.6      | 1.7      | 2.3      |
| Sb <sub>2</sub> O <sub>3</sub> |          |          | 0.3      | 0.2      |

To coat sheet steel for example with the frits of Tables II, III and V, it is important that the steel should be carefully cleaned before the frits are applied to the steel. The cleaning consists in boiling the steel in a cleaner

which may be one of a large number of proprietary cleaners now on the market such as Oakite and Wyan-

dotte. This boiling treatment removes grease and dirt.

After the boiling treatment the steel is rinsed with water

and then given a pickling treatment with 6 percent sul-

phuric acid and heated to a temperature of about 140°

F. The pickled steel is then rinsed with water and put

into a nickel dip which is a solution of nickel sulphate

for the purpose of depositing a thin film of nickel on the

surface of the steel. The nickel-dipped steel is then

rinsed again with water to complete the cleaning opera-

tion and is neutralized to remove acid and then dried.

To the dried and cleaned sheet steel then is applied a sur-

face coating of a frit in the form of a slip.

Many metal articles, especially the thicker ferrous

metals, are preferably cleaned by sand blasting being

coated with nickel before having the slips applied thereto.

In Table VI are shown three examples of ground coat

enamel slips.

**GROUND COAT ENAMELS.—PARTS BY WEIGHT***Table VI*

|      |                            |
|------|----------------------------|
| 100  | Frit (a).                  |
| 2    | Sodium silicate (N-brand). |
| 30   | 1 Borax.                   |
| 30   | Water.                     |
| 100  | 16½ frit (f).              |
| 35   | 33½ frit (d).              |
| ½    | 50 frit (b).               |
| ½    | Refined bentonite.         |
| 30   | Urea.                      |
| 4    | Water.                     |
| 4    | Methanol.                  |
| 100  | Parts frit (a).            |
| 11.1 | Parts titanium dioxide.    |
| 25   | Parts water.               |
| 4    | Parts methanol.            |

These frits are prepared by a smelting operation in which the dry ingredients shown in Table I are mixed together and then heated in a furnace at a temperature of 1800° to 2100° F. to melt the ingredients and then the molten materials are discharged into a body of water or passed through water-cooled rolls to solidify the frits in the form of granular glass. The granular glass frits are then treated to form the slips shown in Table VI by grinding in a water or vehicle suspension to a finely ground material. The grinding is preferably carried out in a ball mill. The fluids, such as water and methanol and sodium silicate, are added to the ingredients as part of the milling charge of the ball mill.

Also coloring pigments such as cobalt-chrome-iron, black cobalt oxide, nickel oxide, iron oxide, copper oxide, and opacifiers, such as titanium dioxide and zirconium oxide to the extent of 0.5 to 10.0% by weight of the frit are added to the frits as they are being prepared as slips. The preparation of the slips provides a suspension of the oxides in water, alcohol, and silicates to have a consistency such that the slip may be applied to the steel plates or articles with a spray gun to obtain a coating by spraying. Furthermore the slip may be painted on the steel plate, or the plate may be coated by dipping. After the coat has been applied to cover the entire surface which is to be enameled, the object is placed in a dryer at about 200-250° F. to remove all volatiles and then placed in a furnace and heated at a temperature of 850° to 1100° F. for a period of two to sixty minutes for the purpose of fusing and maturing the slip or frit coating to the point where it is fused and forms a uniform coating which is bonded to the ferrous articles. Thereupon the

enameled ferrous plate or article may be removed from the furnace and cooled.

Most metal plates have a ground enamel coat and one or several cover coats. One enamel ground coat with one enamel cover coat are often used in coating ferrous articles which provide a very satisfactory coating. The cover coats are made into slips to prepare them for application to the coated material. Examples of three different cover coat slips are shown in Table VII.

#### COVER COAT ENAMELS.—PARTS BY WEIGHT

Table VII.

|     |                    |
|-----|--------------------|
| 100 | Frit (A).          |
| 10  | Titania.           |
| 1/4 | Refined bentonite. |
| 1/2 | Urea.              |
| 35  | Water.             |
| 100 | Frit (B).          |
| 10  | Titania.           |
| 1   | Coloring oxide.    |
| 30  | Water.             |
| 4   | Methanol.          |
| 100 | Frit (A).          |
| 5   | Black oxide.       |
| 1/2 | Refined bentonite. |
| 1/4 | Urea.              |
| 30  | Water.             |
| 5   | Methanol.          |

The cover slips are made in the same way that the ground coat slips are made by grinding the frits shown in Table V with the ingredients shown in the table and water with methanol to form suspensions to be used for placing the coating on a metal sheet having an under coat. The sheet to which an under coat has been applied is sufficiently clean to directly receive the cover coat and one or more coats may be applied to the under coat in building up a final enamel coating of the desired thickness. It is preferred to apply a series of thin coatings one after another in building up the desired enamel surface rather than to use a thick application in an attempt to build up a thick enamel coating in a single operation.

It will be seen from Table II and V that the compositions of the ground and cover coats vary somewhat in order to obtain a uniform bonded coating. The maturing temperature used is sufficiently high so that fusions of the slip occurs in uniting the slip to a metal or to an enamel coating on the metal.

The nature of the slips vary in obtaining hard, soft and medium hard coatings. The composition also is varied in order to adapt the frits and slips for being bonded at different temperatures. If a thin coating is to be applied to a thin metal sheet it is important to have a slip provide a finished composition which will have a thermal linear coefficient of expansion within plus or minus  $1 \times 10^{-6}$  of the coefficient of expansion of the steel to which it is to be applied. If this relationship exists between the coefficients of expansion of the steel and the slip then the coated steel sheet may be bent or flexed repeatedly and the coating will be sufficiently flexible so that it will not chip off when the steel is bent to a comparatively sharp angular condition.

The patents to Deyrup 2,338,099 and 2,467,114 disclose vitreous enamel frits which are applied to glass ware and aluminum at temperatures respectively of 1150° and between 920° and 980° F. The glass forming constituents of which these frits are made are in many respects the same as the constituents used in making the frits of the present invention. A large series of tests have been carried out when using the frits of these patents at the temperatures specified in the patents to learn whether these frits were suitable or could be used for applying a satisfactory vitreous enamel coating to steel. It was found that regardless of the temperatures used for maturing the frits on steel, or ferrous metals having a coefficient of linear expansion below  $14 \times 10^{-6}$ , that satisfactory coatings could not be obtained. In all

cases the fused coatings chipped off or the coatings contained so many fine and large checks that the coated articles were not acid, alkali or moisture proof. The patents define critical relationships of the alkali metal oxides to the sum of silica and titania contents of the frits which appear to apply only to glass and aluminum. These frits are not applicable to ferrous alloys such as steel, cast iron, wrought iron and stainless steel, alloys which have a thermal coefficient of linear expansion much lower than the coefficient of linear expansion of aluminum and much higher than the linear coefficients of expansion of glassware.

The formulae outlined in Tables I and II are critical in obtaining thin flexible coatings that are firmly bonded to the metal and mature into continuous completely covering coatings. The variations which are allowable are quite small to provide for hard, soft and medium hard coatings and to provide for different firing temperatures.

20 In making up the frits the ingredients commonly used are sodium, and potassium carbonates and nitrates, lithium carbonate, titanium dioxide, antimony trioxide, copper oxide, calcium oxide, magnesia, zirconium oxide, lead oxides, dehydrated borax, calcium and sodium fluorides, alumina, phosphorus pentoxide, barium oxide, zinc oxide, and cobalt oxide ( $Co_3O_4$ ). These ingredients are fused together in making the frits and the analyses are expressed as oxides or as molecular fluorine in the tables.

25 The trade is now using special low carbon steels for the manufacture of articles that are being enameled at temperatures above 1400° F. The enamel frits of the present invention may be easily applied to any type of steel, cast and wrought iron, and stainless steels whether 30 the ferrous articles are thick or thin. Thus the enamel and the method of enameling of the present invention are applicable to a large number of metal articles that could not be enameled heretofore.

The preferred form of the invention having been thus 35 described, what is claimed as new is:

1. A low temperature porcelain enamel under coating frit adapted to be bonded to ferrous metal alloys having a coefficient of linear expansion below  $14 \times 10^{-6}$ , said frit having a fusing and maturing temperature between 850° and 1100° F., which comprises a mixture expressed from analysis containing mol. percentages of  $Na_2O$  13.9 to 17.3,  $K_2O$  0.4 to 3.0,  $B_2O_3$  7.5 to 13.1,  $SiO_2$  33.4 to 38.7,  $CaO$  1.0 to 15.6, and the balance of at least one or more of the metal oxides of the group consisting of  $Li_2O$ ,  $CuO$ ,  $MgO$ ,  $TiO_2$ ,  $PbO$ ,  $Al_2O_3$ ,  $BaO$ ,  $ZrO$ ,  $P_2O_5$ ,  $NiO$ ,  $Co_3O_4$  and fluorides.

2. A low temperature porcelain enamel under coating frit as in claim 1 adapted to be bonded to ferrous metal alloys having a coefficient of linear expansion below  $14 \times 10^{-6}$ , said frit having a fusing and maturing temperature between 850° and 1100° F., and which comprises a mixture which expressed from analysis contains metal oxides in the mol percent of the group consisting of

|              |              |
|--------------|--------------|
| $Na_2O$      | 13.9 to 17.3 |
| $K_2O$       | 0.4 to 3.0   |
| $Li_2O$      | 0.0 to 6.0   |
| $B_2O_3$     | 7.5 to 13.1  |
| $SiO_2$      | 33.4 to 38.7 |
| $TiO_2$      | 0.0 to 4.2   |
| 55 $PbO$     | 0.0 to 14.0  |
| $MgO$        | 0.0 to 13.5  |
| $CaO$        | 1.0 to 15.6  |
| $BaO$        | 0.0 to 5.2   |
| $Al_2O_3$    | 0.0 to 0.6   |
| 70 $CuO$     | 0.0 to 3.2   |
| $NiO$        | 1.0 to 1.6   |
| $Co_3O_4$    | 0.0 to 0.2   |
| $ZrO$        | 0.0 to 3.0   |
| $P_2O_5$     | 0.0 to 0.5   |
| 75 and $F_2$ | 0.0 to 8.3   |

3. A low temperature porcelain enamel frit adapted to cover coat ferrous metal alloys having a ground coat as defined in claim 2, said cover coat frit having a coefficient of linear expansion between  $12$  and  $14 \times 10^{-6}$  and a fusing and maturing temperature between  $850^\circ$  and  $1100^\circ$  F., which comprises a mixture expressed from analysis containing mol percentages of

|                                |              |    |
|--------------------------------|--------------|----|
| Na <sub>2</sub> O              | 11.2 to 15.2 | 10 |
| K <sub>2</sub> O               | 1.4 to 2.0   |    |
| Li <sub>2</sub> O              | 4.6 to 6.0   |    |
| B <sub>2</sub> O <sub>3</sub>  | 8.1 to 10.0  |    |
| SiO <sub>2</sub>               | 28.9 to 36.5 |    |
| F <sub>2</sub>                 | 0.0 to 12.4  | 15 |
| TiO <sub>2</sub>               | 2.0 to 6.1   |    |
| PbO                            | 10.9 to 14.2 |    |
| MgO                            | 8.1 to 12.7  |    |
| CaO                            | 0.0 to 1.7   |    |
| BaO                            | 1.7 to 6.6   | 20 |
| Sb <sub>2</sub> O <sub>3</sub> | 0.0 to 0.3   |    |

4. The low temperature porcelain enamel frit as defined in claim 2 to which a ceramic pigment in an amount from 0.5% to 10% is added to obtain desired colors.

5. A process of making a porcelain enamel ferrous metal alloy article having a coefficient of linear expansion in the range of  $12$  to  $14 \times 10^{-6}$ , comprising removing grease, rust, scale and moisture from the surface to be coated, applying a uniform coating of a slip formed with a ground fused mixture of a frit as defined in claim 2 having a coefficient of linear expansion within  $\pm 1 \times 10^{-6}$  of the coefficient of linear expansion of the ferrous metal alloy used, then heating the coated metal alloy article to a temperature in the range of  $850^\circ$  to  $1150^\circ$  F. for a sufficient period of 2 to 30 minutes to fuse and mature the slip enamel surface to a continuous bonded coating.

6. The process as defined in claim 5 wherein a cover coating of a slip formed from a frit as defined in claim 3 is applied, then heating the coated metal in the temperature range of  $850^\circ$  to  $1100^\circ$  F. to fuse and mature the cover coating to obtain a continuous bonded enamel surface.

7. The process as defined in claim 6 wherein the thickness of slip coating is between 1 to 3 mils of enamel thickness.

8. The process as defined in claim 6 wherein the thickness of enamel coating is within the range of  $1\frac{1}{2}$  to 15 grams per square foot of coated surface.

9. A low temperature porcelain enamel frit for bonding as under coat to ferrous metal alloys having a coefficient of linear expansion between  $12 \times 10^{-6}$  and  $14 \times 10^{-6}$  and for fusing and maturing as a continuous bonded surface at temperatures between  $850^\circ$  and  $1100^\circ$  F. comprising mol. percentages of

|                               |      |    |
|-------------------------------|------|----|
| Na <sub>2</sub> O             | 15.0 | 60 |
| K <sub>2</sub> O              | 2.0  |    |
| Li <sub>2</sub> O             | 6.0  |    |
| B <sub>2</sub> O <sub>3</sub> | 8.0  |    |
| SiO <sub>2</sub>              | 35.7 |    |
| TiO <sub>2</sub>              | 2.0  | 65 |
| PbO                           | 14.0 |    |
| MgO                           | 12.5 |    |
| CaO                           | 1.7  |    |
| CuO                           | 2.0  |    |
| NiO                           | 1.1  | 70 |

10. A low temperature porcelain enamel frit for bonding as an under coat to ferrous metal alloys having a coefficient of linear expansion between  $12 \times 10^{-6}$  and  $14 \times 10^{-6}$  and for fusing and maturing as a continuous

bonded coating at temperatures between  $850^\circ$  and  $1100^\circ$  F. comprising mol. percentages of

|                               |      |
|-------------------------------|------|
| Na <sub>2</sub> O             | 13.9 |
| K <sub>2</sub> O              | 1.9  |
| Li <sub>2</sub> O             | 5.5  |
| B <sub>2</sub> O <sub>3</sub> | 11.7 |
| SiO <sub>2</sub>              | 33.4 |
| TiO <sub>2</sub>              | 2.8  |
| PbO                           | 13.0 |
| MgO                           | 13.5 |
| CaO                           | 1.5  |
| CuO                           | 1.8  |
| NiO                           | 1.0  |

11. A low temperature porcelain enamel frit for bonding as an undercoat to ferrous metal alloys having a coefficient of linear expansion between  $12 \times 10^{-6}$  and  $14 \times 10^{-6}$  and for fusing and maturing as a continuous bonded coating at temperatures between  $850^\circ$  and  $1100^\circ$  F. comprising mol. percentages of

|                               |      |
|-------------------------------|------|
| Na <sub>2</sub> O             | 15.0 |
| K <sub>2</sub> O              | 2.0  |
| Li <sub>2</sub> O             | 6.0  |
| B <sub>2</sub> O <sub>3</sub> | 8.0  |
| SiO <sub>2</sub>              | 36.0 |
| TiO <sub>2</sub>              | 2.0  |
| PbO                           | 14.0 |
| MgO                           | 8.0  |
| CaO                           | 1.0  |
| BaO                           | 5.0  |
| CuO                           | 3.0  |

35 12. A low temperature porcelain enamel frit for bonding as an under coat to ferrous metal alloys having a coefficient of linear expansion between  $12 \times 10^{-6}$  and  $14 \times 10^{-6}$  and for fusing and maturing as a continuous bonded coating at temperatures between  $850^\circ$  to  $1100^\circ$  F. comprising mol. percentages of

|                               |      |
|-------------------------------|------|
| Na <sub>2</sub> O             | 16.3 |
| K <sub>2</sub> O              | 3.0  |
| Li <sub>2</sub> O             | 5.2  |
| B <sub>2</sub> O <sub>3</sub> | 8.1  |
| SiO <sub>2</sub>              | 38.1 |
| TiO <sub>2</sub>              | 4.2  |
| PbO                           | 12.4 |
| MgO                           | 8.8  |
| CaO                           | 1.1  |
| CuO                           | 2.8  |

55 13. A low temperature porcelain enamel frit for bonding as an under coat to ferrous metal alloys having a coefficient of linear expansion between  $12 \times 10^{-6}$  and  $14 \times 10^{-6}$  and for fusing and maturing as a continuous bonded coating at temperatures between  $850^\circ$  and  $1100^\circ$  F. comprising mol. percentages of

|                               |      |
|-------------------------------|------|
| Na <sub>2</sub> O             | 14.9 |
| K <sub>2</sub> O              | 2.8  |
| Li <sub>2</sub> O             | 4.8  |
| B <sub>2</sub> O <sub>3</sub> | 7.5  |
| SiO <sub>2</sub>              | 35.3 |
| F <sub>2</sub>                | 3.7  |
| TiO <sub>2</sub>              | 3.9  |
| PbO                           | 11.5 |
| MgO                           | 8.2  |
| CaO                           | 4.8  |
| CuO                           | 2.6  |

75 14. A low temperature porcelain enamel frit for bonding as an under coat to ferrous metal alloys having a coefficient of linear expansion between  $12 \times 10^{-6}$  and  $14 \times 10^{-6}$  and for fusing and maturing as a continuous

bonded coating at temperatures between 850° and 1100° F. comprising mol. percentages of

|                                |      |    |
|--------------------------------|------|----|
| Na <sub>2</sub> O              | 16.4 | 5  |
| K <sub>2</sub> O               | 0.4  |    |
| Al <sub>2</sub> O <sub>3</sub> | 0.6  |    |
| B <sub>2</sub> O <sub>3</sub>  | 13.1 |    |
| SiO <sub>2</sub>               | 35.1 |    |
| F <sub>2</sub>                 | 8.3  | 10 |
| CaO                            | 15.6 |    |
| BaO                            | 5.2  |    |
| ZrO                            | 3.0  |    |
| P <sub>2</sub> O <sub>5</sub>  | 0.5  |    |
| NiO                            | 1.6  | 15 |
| Co <sub>3</sub> O <sub>4</sub> | 0.2  |    |

15. A low temperature porcelain enamel frit for bonding as an under coat to ferrous metal alloys having a coefficient of linear expansion between  $12 \times 10^{-6}$  and  $14 \times 10^{-6}$  and for fusing and maturing as a continuous bonded coating at temperatures between 850° and 1100° F. comprising mol. percentages of

|                               |      |    |
|-------------------------------|------|----|
| Na <sub>2</sub> O             | 17.3 |    |
| K <sub>2</sub> O              | 1.7  |    |
| Li <sub>2</sub> O             | 2.6  |    |
| B <sub>2</sub> O <sub>3</sub> | 10.0 |    |
| SiO <sub>2</sub>              | 38.7 |    |
| F <sub>2</sub>                | 4.7  | 30 |
| TiO <sub>2</sub>              | 2.1  |    |
| PbO                           | 6.0  |    |
| CaO                           | 9.0  |    |
| BaO                           | 3.0  |    |
| ZrO                           | 1.7  |    |
| CuO                           | 3.2  |    |

16. A low temperature porcelain enamel frit for use as a cover coat over an under coat bonded to the face of a ferrous alloy article, said frit having a fusing and maturing temperature between 850° F. to 1100° F. comprising mol. percentages as follows:

|                               |      |    |
|-------------------------------|------|----|
| Na <sub>2</sub> O             | 15.2 |    |
| K <sub>2</sub> O              | 2.0  | 45 |
| Li <sub>2</sub> O             | 6.0  |    |
| B <sub>2</sub> O <sub>3</sub> | 8.1  |    |
| SiO <sub>2</sub>              | 36.5 |    |
| TiO <sub>2</sub>              | 2.0  |    |
| PbO                           | 14.2 | 50 |
| MgO                           | 12.7 |    |
| CaO                           | 1.7  |    |
| BaO                           | 1.6  |    |

17. A low temperature porcelain enamel frit for use as a cover coat over an under coat bonded to the face of a ferrous alloy article, said frit having a fusing and maturing temperature between 850° F. and 1100° F. comprising mol. percentages as follows:

ing temperature between 850° F. and 1100° F. comprising mol. percentages as follows:

|                               |      |  |
|-------------------------------|------|--|
| Na <sub>2</sub> O             | 15.2 |  |
| K <sub>2</sub> O              | 2.0  |  |
| Li <sub>2</sub> O             | 6.0  |  |
| B <sub>2</sub> O <sub>3</sub> | 8.2  |  |
| SiO <sub>2</sub>              | 36.5 |  |
| TiO <sub>2</sub>              | 2.0  |  |
| PbO                           | 14.2 |  |
| MgO                           | 8.1  |  |
| CaO                           | 1.2  |  |
| BaO                           | 6.6  |  |

18. A low temperature porcelain enamel frit for use as a cover coat over and under coat bonded to the face of a ferrous alloy article, said frit having a fusing and maturing temperature between 850° F. and 1100° F. comprising mol. percentages as follows:

|                                |      |  |
|--------------------------------|------|--|
| Na <sub>2</sub> O              | 15.1 |  |
| K <sub>2</sub> O               | 2.0  |  |
| Li <sub>2</sub> O              | 6.0  |  |
| B <sub>2</sub> O <sub>3</sub>  | 8.1  |  |
| SiO <sub>2</sub>               | 36.4 |  |
| TiO <sub>2</sub>               | 2.0  |  |
| PbO                            | 14.1 |  |
| MgO                            | 12.7 |  |
| CaO                            | 1.7  |  |
| BaO                            | 1.7  |  |
| Sb <sub>2</sub> O <sub>3</sub> | 0.3  |  |

19. A low temperature porcelain enamel frit for use as a cover coat over an under coat bonded to the face of a ferrous alloy article, said frit having a fusing and maturing temperature between 850° F. and 1100° F. comprising mol. percentages as follows:

|                                |      |  |
|--------------------------------|------|--|
| Na <sub>2</sub> O              | 11.2 |  |
| K <sub>2</sub> O               | 1.4  |  |
| Li <sub>2</sub> O              | 4.6  |  |
| B <sub>2</sub> O <sub>3</sub>  | 10.0 |  |
| SiO <sub>2</sub>               | 28.9 |  |
| F <sub>2</sub>                 | 12.4 |  |
| TiO <sub>2</sub>               | 6.1  |  |
| PbO                            | 10.9 |  |
| MgO                            | 12.0 |  |
| BaO                            | 2.3  |  |
| Sb <sub>2</sub> O <sub>3</sub> | 0.2  |  |

#### References Cited in the file of this patent

#### UNITED STATES PATENTS

|           |                  |               |
|-----------|------------------|---------------|
| 1,496,505 | Whittaker et al. | June 3, 1924  |
| 1,783,740 | McKeown          | Dec. 2, 1930  |
| 2,004,632 | Martin           | June 11, 1935 |
| 2,175,689 | Gallup et al.    | Oct. 10, 1939 |
| 2,321,656 | Chester          | June 15, 1943 |
| 2,467,114 | Deyrup           | Apr. 12, 1949 |
| 2,660,531 | Fraser et al.    | Nov. 24, 1953 |

UNITED STATES PATENT OFFICE  
CERTIFICATE OF CORRECTION

Patent No. 2,842,458

July 8, 1958

Edward J. Feeney et al.

It is hereby certified that error appears in the printed specification of the above numbered patent requiring correction and that the said Letters Patent should read as corrected below.

Column 2, Table I, first column thereof, line 9, for "PbO<sub>2</sub>" read  
-- PbO --; same table and column, line 13, for "ZnO" read -- ZrO --; column 3, Table II, first column thereof, line 13, for "ZnO" read -- ZrO --; same column, Table III, first column thereof, line 9, for "TiO" read -- TiO<sub>2</sub> --; same table and column, line 10, for "PbO<sub>2</sub>" read -- PbO --; same column 3, Table IV, fourth column thereof, under the heading "C", lines 8 to 12, opposite "PbO" for "14.1" read -- 38.1 --; opposite "MgO" for "12.7" read -- 6.1 --; opposite "CaO" for "1.7" read -- 1.1 --; opposite "BaO" for "1.7" read -- 2.9 --; opposite "Sb<sub>2</sub>O<sub>3</sub>" for "0.3" read -- 1.0 --; column 5, line 51, before "applied" insert -- be --.

Signed and sealed this 4th day of November 1958.

(SEAL)

Attest:

KARL H. AXLINE

Attesting Officer

ROBERT C. WATSON  
Commissioner of Patents